

## UNITED STATES PATENT OFFICE

JOSEPH NÜSSLEIN, OF LUDWIGSHAFEN-ON-THE-RHINE, GERMANY, ASSIGNOR TO I. G. FARBEININDUSTRIE AKTIENGESELLSCHAFT, OF FRANKFORT-ON-THE-MAIN, GERMANY, A CORPORATION OF GERMANY

## TREATING FIBROUS MATERIALS OR TEXTILES

No Drawing. Application filed January 22, 1926, Serial No. 83,143, and in Germany January 21, 1925.

In many operations or processes to which fibrous materials or textiles are subjected, the difficulty arises that the materials are not uniformly or not sufficiently or too slowly 5 wetted or penetrated by the preparation or liquid applied to the said materials. In some cases the use of soap has more or less overcome these difficulties, but in other cases and particularly in sizing no means to over- 10 come them have been suggested.

I have now found that in sizing operation, the said difficulties can be overcome by the addition of organic sulfonic acids which may be used either as such or in the state of salts. 15 Such sulfonic acids may belong to the aliphatic series such as sulfonated brown coal tar oils, or more suitably to the aromatic series. Among the latter, in general, those containing side chains have been found to be 20 most suitable. I may mention as examples of compounds especially suitable for these purposes propyl and butyl derivatives of naphthalene sulfonic acids, also aromatic sulfonic acids substituted by alkylated amino 25 groups, for example dimethyl metanilic acid, diethyl-alpha-naphthylamine sulfonic acid or similar compounds, or other salts. Condensation products of sulfonated phenols or 30 naphthalene and formaldehyde may also be mentioned.

Such sulfonic acids may be used with great advantage in sizing wool, cotton, jute, leather, hair, rayon or artificial silk, paper or other fibrous material of vegetable, ani- 35 mal or artificial origin, or textiles or other articles made thereof.

The sulfonic acids may be employed in connection with other additions, including soap or saponaceous materials.

40 In sizing operations, the sulfonic acids or their salts may be added to the sizing compound such as glue, gelatine, starch, dextrine or other suitable materials. For example a composition for sizing warps, especially cotton warps is prepared by adding to one litre of water, from 10 to 20 grammes of potato starch and a solution of from 3 to 8 grammes of butylated naphthalene sulfonic acid sodium salt (obtainable by condensing a naphthalene sulfonation mixture with normal 45 50

butyl alcohol at an elevated temperature) in hot water and boiling for 15 minutes.

My invention is, however, not restricted to the above examples.

I do not lay claim in this application to 55 the process of fulling and to preparations for carrying out this process, such being claimed, in my divisional application Ser. No. 129,087, filed Aug. 13th, 1926 simultaneously with this amendment.

60 In the appended claims the term "sulfonate" embraces sulfonic acids which for the purpose of this invention are considered hydrogen sulfonates.

65 Now what I claim is:

1. A preparation suitable for sizing textile materials which comprises a practically water-soluble sizing material and a water-soluble compound of an alkylated aromatic sulfonic acid.

70 2. A preparation suitable for sizing textile materials which comprises a practically water-soluble sizing material and a water-soluble salt of a naphthalene sulfonic acid substituted by an alkyl radicle selected from 75 alkyl radicles containing from 3 to 4 carbon atoms.

3. A preparation suitable for sizing textile materials which comprises from 10 to 30 80 grams of potato starch and from 3 to 8 grams of the sodium salt of a butylated naphthalene sulfonic acid.

85 In testimony whereof I have hereunto set my hand.

JOSEPH NÜSSLEIN. 85

90

95

100